

April 7, 1931.

H. B. LEARY, JR

1,800,146

PROCESS OF MARKING FIBROUS MATERIAL

Filed June 27, 1930

FIG. 1.



FIG. 2.



FIG. 3.



FIG. 4.



FIG. 5.



FIG. 6.



Inventor

H. B. Leary, Jr.

234

Motion, Cont., Morse & Grindle  
Attorneys

## UNITED STATES PATENT OFFICE

HARRY BURTON LEARY, JR., OF WASHINGTON, DISTRICT OF COLUMBIA

## PROCESS OF MARKING FIBROUS MATERIAL

Application filed June 27, 1930. Serial No. 464,351.

This invention relates to the treatment of fibrous material, such as wood, to form markings of any desired configuration thereon, and has for its principal object the provision of a new and improved method whereby such material may be permanently marked without disfiguring or interrupting the continuity or smoothness of the surface of the material.

10 A more specific object of the invention is the provision of a process of treating fibrous material to impart the appearance of pronounced and attractive grain to the surface thereof without the use of paints or 15 pigments of contrasting color.

A further object of the invention is the provision of a piece or sheet of fibrous material for use in structural or decorative work in which a portion of the fibers adjacent the surface of the material are deformed in a manner not instantly apparent to the observer but which may be made clearly visible by the application of a light-pervious coating, such as varnish, to afford 25 a design distinctive in appearance.

Further objects and features of the invention will be apparent from the following description of the invention taken in connection with the accompanying drawings, in which:

Figure 1 is a plan view of a piece of fibrous material to which the process may be applied;

Figure 2 is a corresponding plan view 35 showing the same piece of material after completion of the initial step of deforming the fibers adjacent the surface to provide the desired markings or design;

Figure 3 is a section on the line 3—3 of 40 Figure 2;

Figure 4 is a section corresponding to Figure 3 and illustrating a further step in the process;

Figure 5 is a sectional view showing the 45 material with the light-pervious coating applied to the surface thereof; and

Figure 6 is a plan view of the finished piece of material.

When a light-pervious coating, such as 50 varnish, is applied to the surface of wood

or other fibrous material bearing a pronounced grain, the effect of the grain is intensified. This intensification of the grain is probably due in part to the fact that the fibers of the material are somewhat distorted or altered in direction at those points where grain appears, this being particularly true where knots or other irregularities appear in the surface of the material; the varnish or other coating is absorbed to a greater extent by reason of the looseness and irregularity of the fibers at such points, the density of the coating being correspondingly increased.

At any rate, it is unquestionably true that 65 the application of varnish to a grained surface serves to emphasize the grain primarily by reason of the distortion or irregularity of the fibers, and I propose to utilize this principle for the purpose of providing artificial graining or other marking of wood and similar fibrous materials by first deforming the fibers adjacent the surface and thereafter applying a coating of varnish or similar material.

I have also found that when fibrous material is indented by the application of pressure, the fibers are distorted, not only laterally of the indented portion but beneath the indentation so that the removal of the 80 surface to the depth of or slightly below the indentation does not entirely remove the distorted fibers, those fibers beneath the indented portion remaining distorted and being intensified in appearance by the application of varnish thereto.

Referring now specifically to the drawings, it will be observed that the block or piece 10 of material to be treated, illustrated in Figure 1 as having fibers extending generally in the same direction, is subjected to pressure at various points on the surface to depress or indent portions of the surface in the manner shown in Figure 2. 85 These indented portions may assume any desired form, the indentations 12 being effected for the purpose of obtaining a pronounced grain effect and the indentations indicated at 13 comprising a design such as 95 100

might be desirable for decorative or advertising purposes.

Figure 3 is a sectional view through the piece of material and illustrates the manner in which the indentations are produced and the probable manner of distortion of the fibers. The rounded indentations intended to give the appearance of pronounced grain are preferably produced by an instrument having a blunt or rounded head adapted to be driven into the surface. In lieu of such an instrument, the desired indentations may be produced by driving or firing a small round shot such as is commonly used in air rifles into the surface of the material. The shape of the instrument may also be so chosen as to produce a design having extended curved or straight lines as distinguished from the point indentations such as are suitable to represent grain in the material. It will be appreciated that the indentations might be produced by means of a tool having a design such as represented at 13 produced in its entirety in relief on the face thereof and adapted to be stamped or driven into the surface of the material.

It will be observed that the fibers of the material are distorted not only on the sides of the depressed or indented portion but also beneath the indented portion, these fibers being given a permanent set by the application of pressure or force through the medium of the indenting tool.

Figure 4 is a sectional view illustrating a further step in the process, a portion of the surface of the material having been removed to the depth of the indentations or slightly beneath the bottom of the indented portions to provide a smooth surface. In the event that the process is applied to wood, the surface may be readily removed by planing or abrading to the desired depth, and the appearance of the material is substantially that illustrated in Figure 1, the deformation of the fibers at certain points on the surface being not immediately apparent to the observer.

A coating of light-pervious material is now applied to the smooth surface, any conventional varnish being found suitable for the purpose, and as pointed out above, the distorted fibers are intensified in appearance so that the indented portions illustrated in Figure 2 are plainly reproduced and appear somewhat darker than the surrounding untreated surface of the material. The light-pervious coating is indicated at 16 in Figure 5 in which the deformation of the fibers immediately beneath the coating at certain points in the surface of the material has been shown.

The plan view of the finished product is represented in Figure 6, the configurations in design and the markings in imitation of grain being quite pronounced and appear-

ing as a natural formation of the fibrous material as distinguished from the more conventional printed or impressed markings. The finished surface is smooth and uninterrupted and the markings are permanent and can only be removed by removing the varnish and the partially deformed surface of the material.

It will be appreciated that the depth to which the surface of the material is removed will depend largely on the nature of the material and the effect which it is desired to produce. For instance, in the treatment of some woods it is found that removal of the surface only to the depth of the depression or indentation is insufficient since the fibers immediately beneath the point of indentation are so distorted that they absorb considerable varnish and are caused to swell, thereby impairing the smooth finish of the resulting surface. Under such circumstances it is necessary to remove the surface and a sufficient portion of the distorted fibers to insure a perfect finish and freedom from subsequent swelling of the fibers. Furthermore, by varying the depth to which the surface is removed, varying degrees of intensification of the marking or design may be obtained, since the extent of distortion of the fibers is greatest near the surface and decreases toward the interior of the material.

It is also obvious that a novel effect may be obtained by distorting the fibers over the entire surface or over a considerable portion of the surface. If the fibers over the entire surface of the material are distorted, the appearance of the finished material will depend on the uniformity of distortion of the fibers and the depth to which the distorted fibers are removed prior to the application of the varnish.

While I have illustrated a representation of grain in the material by the production of isolated markings, it will be apparent that the applied design may assume any form. For instance, indentations in the shape of broken, curved, or wavy lines such as frequently appear in highly grained woods may be produced and striking natural effects closely approximating the original wood grain may be obtained.

Such further alterations and modifications of the process described herein are contemplated as fall within the spirit and scope of the appended claims.

Having thus described the invention, what is claimed as new and desired to be secured by Letters Patent is:

1. A process of treating fibrous material to produce markings thereon, which comprises indenting the surface of the material, removing the surface to a depth sufficient to expose the distorted fiber beneath the in-

dentation, and applying a light-pervious coating to the resulting surface.

2. A process of treating fibrous material to produce markings thereon, which comprises applying pressure to produce indentation of the surface of the material, removing the surface to a depth sufficient to expose the distorted fiber beneath the indentation, and applying a light-pervious

10 varnish to the surface thus formed.

3. A process of treating fibrous material to produce markings thereon, which comprises distorting the fibers of the material, removing the surface of the material to the 15 depth of apparent distortion, and coating the surface thus formed with a light-pervious varnish.

4. A process of treating wood to produce the effect of grain thereon, which comprises 20 indenting the surface of the wood, planing the surface sufficiently to remove the indented portion without removing all of the distorted fiber beneath the indentation, and coating the surface thus formed with a 25 transparent varnish.

5. As an article of manufacture, a piece 30 of wood having a smooth flat surface coated with a varnish, portions of the fibers of the wood adjacent said surface being distorted to give the appearance of markings when viewed through the varnish.

6. As an article of manufacture, a piece 35 of wood having a smooth flat surface coated with a varnish, the fibers of the wood immediately beneath the varnish coating being distorted to alter the appearance of the varnished surface.

7. A process of treating fibrous material which consists in distorting the fibers adjacent 40 the surface, removing such portion of the fibers as are distorted to such an extent as to swell on the application of liquid thereto, and applying a liquid coating to the surface.

45 In testimony whereof I hereunto affix my signature.

HARRY BURTON LEARY, Jr.